

# UNITED STATES PATENT OFFICE.

CHARLES PLEASANTS MEBANE, OF CLEVELAND, OHIO, ASSIGNOR, BY MESNE ASSIGNMENTS, TO EDWIN C. HENN, OF CLEVELAND, OHIO, A CORPORATION OF OHIO.

## CARBONIZING COMPOUND AND PROCESS OF MAKING THE SAME.

1,310,918.

Specification of Letters Patent.

Patented July 22, 1919.

No Drawing.

Application filed June 7, 1917. Serial No. 173,430.

*To all whom it may concern:*

- Be it known that I, CHARLES P. MEBANE, a citizen of the United States, residing at Cleveland, in the county of Cuyahoga and 5 State of Ohio, have invented certain new and useful Improvements in Carbonizing Compounds and Processes of Making the Same, of which the following is a specification.
- 10 This invention relates to an improved process for carburizing steel and has for its general object to accomplish this result in an improved, economical and efficient manner.
- 15 A further object is the provision of a carbonizing material or composition of matter whereby this process may be carried out and which after each operation the portion deteriorated is removed and new energizer 20 added.
- The carburizing operation as ordinarily conducted consists generally in making a mixture of a carbonaceous material and an energizer such as sodium carbonate, 25 barium carbonate, etc., and in embedding the article to be carburized in this mixture and subjecting the article and the mixture to a temperature which will result in adding to the article the amount of carbon necessary to secure the desired degree of hardness in the outer film or layer of the metal 30 after quenching. At the end of the carburizing operation the greater portion of the material is left unconsumed and may be used 35 in succeeding operations. However, the carbonate will be present in insufficient quantities to secure a maximum efficiency in the succeeding uses of the mixture as the energizer gradually loses its strength and 40 after a number of usages ceases to act and a large portion of the carbonaceous material has to be thrown away. In some cases new material is added each time it is used. This is to give additional strength and it is true 45 that fair commercial results are obtained. This material, however, commercially speaking, will give about 75% efficiency as compared with new material.
- It has been attempted to correct this decreasing efficiency by adding a fresh supply 50 of energizer to the mixture after each succeeding operation. This, however, has been attended with a serious objection that the metal thus treated is very apt to be pitted or 55 spotted while a glassy residue forms in the
- boxes eventually filling them up and the carburized parts are not uniform throughout. It has also been proposed to make a mixture of charcoal and an energizer in proper proportions and to keep this mixture on hand; this, however, has been attended with the objection that the agitation of the mixture as through the shaking or jarring of the building by the operation of machinery, etc., even though slight, is sufficient to separate the heavier energizer and the light carbonaceous matter with the result that the mixture does not remain homogeneous. The energizer accumulating at the lower part or bottom of the receptacle containing the mixture while the carbonaceous matter remaining at the upper part of the said receptacle will in time have practically no energizer mingled therewith.
- It is the purpose of this invention to improve the process of carburizing so as to overcome the objections noted herein before while securing the same efficiency in the last carburizing operation as in the first and also to secure these results in a simple and particularly economical manner. In carrying out my invention I take a quantity of wood suitable for a day's work in the particular plant wherein the process may be carried on, said wood being of a size which preferably will pass through a screen having three or four meshes to the lineal inch. This wood is then saturated in a fireproofing solution to which is added an energizer. This fireproofing is obtained for instance by 85 soaking in a fireproofing solution such as silicate of soda, which causes the wood to char and not burn to ash, and which solution also contains the energizer. After this soaking the wood is then dried and ready 90 for use. This fireproof solution and energizer penetrate the pores of the wood and decrease the shrinkage. That is, wood not treated or fireproofed will shrink in volume about 66 2/3% which would uncover the parts 95 in the carburizing boxes and cause them to scale or otherwise spoil them, whereas fireproofed wood holds its shape very well and is practical to use.
- This treated wood is then dried and used 100 as a commercial carburizer.
- After taking the carburizing boxes from the furnace and removing the parts carburized, this carburizer is treated with a solution previously made of water, sodium 105

carbonate and sodium chlorid using about four parts of sodium carbonate to one of sodium chlorid. The density of this solution should be about  $7\frac{1}{2}$  Baumé but is varied according to the amount of carbon required in the case. Any suitable apparatus may be used for applying the solution, such as an old fashioned watering can or other device to sprinkle the fireproofed wood, now charcoal, and hot, with the solution. The heat remaining in the charcoal drives off the moisture and the energizer adheres to the charcoal. This adhering is caused by the sudden contraction of the carbonaceous material. The moisture also kills the fire in the charcoal and prevents a big waste. It will be noted that I do not use any tacky substance nor is the heat in the charcoal sufficient to fuse the chemicals. After the sprinkling operation a considerable quantity of the fireproofed wood, now charcoal, will be left, leaving the energizer in a new, spent and partly spent condition. If this mixture of charcoal and energizer is used repeatedly without sprinkling the metal treated thereby will not be as effectively carburized as in the preceding work when the energizer was in a fresh condition, furthermore, the scale of efficiency of the resultant mixture will diminish from operation to operation with a corresponding diminution in the efficiency of the carburizing accomplished therewith. This condition cannot be corrected as a commercial proposition by adding fresh energizer as the mixing of the fresh energizer with the spent and partly spent energizer results after several operations in spotting or pitting the articles to be carburized also the forming of a glassy substance in the carburizing boxes as well as in lack of uniformity in the carburizing of the articles. This detrimental action is believed to be due to the chemical changes which have been produced in the original energizer. In order to utilize the charcoal and at the same time secure the maximum efficiency in the subsequent re-use of the same or before the particular job of carburizing has been complete I sieve the mass of charcoal and energizer using preferably a  $\frac{1}{64}$  mesh sieve. A sieve of this fineness will separate the detrimental spent energizer from the carbonaceous material leaving the new energizer adhering to the carbonaceous material.

By this process and the carburizing composition employed the carbonaceous material may be re-used producing the same results as before until completely consumed and with no substantial waste of material. The very small amount of carbonaceous material and spent energizer which are discarded by passing through a sieve of  $\frac{1}{64}$  mesh is ex-

tremely cheap. I then take the sieved material and add thereto a sufficient quantity of either wood or charcoal to make a mass as large or larger than the original mass. This is then used the same as any commercial carburizer and upon removal from the furnace is treated as before again producing like results.

This method is the only one by which all of the carbonaceous material can be used without deterioration or detrimental results. Only the very fine dust and chemicals that would fly in the room are thrown away and it is the only way in which the hardener in charge of the room can regulate the amount of the carbon contents in the case. This latter is done by the density of the solution and the amount of the solution sprinkled on the hot charcoal.

Where 20% or more of the work is direct quenched, that is removed from the hardening boxes at a red heat, and the remainder 80% or less is allowed to cool in the boxes, that portion of charcoal remaining from the direct quenched operation can be treated with a solution much denser than  $7\frac{1}{2}$  degrees Baumé and this mixture added to the wood or charcoal in the proportions to secure the desired results.

Whereas in the case of hardening ball bearings and other work that is cooled in the boxes, none being removed therefrom hot, this process is not practical as there is no heat in the carbonaceous substance to cause the moisture to evaporate and for material to be used for this purpose the charcoal can be treated in another place and this treated charcoal added to the untreated wood or charcoal using about one part treated to four parts untreated more or less according to the results desired.

The commercial carburizing material on the market reaches the consumer mixed and the man in charge, termed the hardener, has no control over the amount of carbon injected into the case, by this mixture, as this is chiefly regulated by the amount and kind of energizer used and the amount and kind of carbonaceous material employed. With my method the hardener, by varying the specific gravity of the solution or the amount of the solution, the carbon contents of the case can be increased or decreased at will within limits consistent with good shop practice, as he adds the energizer and has a given carbonaceous material to work on, he can produce any amount of carbon in the case and therefore any degree of hardness. This is of importance as the carbon contents of the case can be varied to suit conditions without varying shop practices which have been found suitable for their requirements. For example:—In shop practice it may be found that to carbonize at 1650 F. and quench direct from the box a suitable core is

produced, but not so with the carbon contents of the case.

The hardener may produce the desired carbon contents by varying the gravity of 5 the solution or amount of solution or both.

In the claims hereto appended I employ the term "fireproof", "fireproofed" or "fire-proofing" in connection with carbonaceous material that has been treated to indicate 10 that it does not shrink in volume when heated as much as it would if not treated, or as much as when bought on the open market.

Having thus described my invention what I claim is:—

15 1. A composition for the purpose specified comprising a mixture of fireproofed carbonaceous material and an energizer including sodium chlorid.

20 2. A composition of matter for the purpose specified comprising an intimate mixture of carbonaceous matter treated so as not to have excess shrinkage, an energizer and finely divided carbonaceous material.

25 3. A composition of matter for the purpose specified comprising fireproofed carbonaceous material, a carbonate and finely divided carbonaceous material, the carbonate being intimately mingled with the carbonaceous material and this mixture being 30 intimately mingled with the fireproofed carbonaceous material.

35 4. A composition of matter for the purpose specified comprising a mixture of fireproofed carbonaceous material, finely divided, fireproofed carbonaceous material and an energizer, the energizer being mingled with and adhering to the fireproofed carbonaceous material.

40 5. A composition of matter for the purpose specified comprising a mixture of two carbonaceous substances either or both of which are fireproofed and an energizer including sodium chlorid.

45 6. A composition of matter for the purpose specified comprising a mixture of fireproofed carbonaceous material sprinkled with a solution containing an energizer, the ingredients being mingled in about the following proportions: Charcoal 100 parts by weight, energizer 1-35 parts by weight.

50 7. A composition of matter for the purpose specified comprising a mixture of carbonaceous material sprinkled with a solution containing sodium carbonate and sodium chlorid being mingled in about the following proportions:—carbonaceous material 100 parts by weight, carbonate 2-35 parts, by weight, chlorid  $\frac{1}{2}$ -10 parts by weight.

60 8. The process of carburizing which consists in heating the article to be carburized in the presence of a mixture of fireproofed carbonaceous material, sodium carbonate, sodium chlorid and additional carbonaceous material and then removing the detrimental

part of the carbonate and chlorid residue after the operation and adding to the hot charcoal a fresh quantity of the solution containing the energizer.

9. The process of preparing carburizing 70 compositions for use and re-use, which consists in sprinkling a hot carbonaceous material with a solution containing an energizer including sodium chlorid, mingling the mixture thus formed with a carbonaceous material, heating the article or articles to be carburized in the presence of the aforesaid mixture, and then after the conclusion of the carburizing and sprinkling operation separating the detrimental spent and partly 80 spent energizer from the carbonaceous material and adding thereto untreated carbonaceous material.

10. The process of preparing carburizing 85 compositions for use and re-use, which consists in sprinkling hot carbonaceous material with a solution containing an energizer including sodium chlorid, mingling the mixture thus formed with other carbonaceous material, heating the article or articles to be carburized in the presence of the aforesaid mixture, and after the conclusion of the aforesaid operation separating the spent or partly spent energizer from the mixture.

11. The process of preparing carburizing 95 composition for use and re-use, which consists in sprinkling hot charcoal with a solution containing an energizer including sodium chlorid in about the proportions specified and after the use of such mixture 100 for the carburizing operation again sprinkling and then sifting the remaining mass to remove therefrom the detrimental spent or partly spent energizer, and thereafter adding to the remainder sufficient wood or charcoal to secure the proper proportions for the succeeding operation.

12. The process of carburizing metal which consists in heating the same in a mixture of fireproofed carbonaceous material 110 and an energizer.

13. The process of preparing a carburizing composition, which consists in treating wood with a fireproofed solution containing an energizer including sodium 115 chlorid, and then drying the so treated material.

14. The process of preparing a carburizing composition, which consists in treating a carbonaceous material with a fireproofed 120 solution containing an energizer, and then drying the so treated material.

15. A composition of matter for the purpose specified comprising fireproofed sawdust and an energizer including sodium 125 chlorid.

16. The process of preparing a carbonizing material which consists in treating wood by saturating it with a fireproofing material and an energizer.

17. The process of preparing a carbonizing material which consists in treating sawdust having a fineness adapted to pass through a screen having three or four meshes to the lineal inch by saturating it with a fireproofing material and an energizer. 5  
 18. The process of preparing a carbonizing material which consists in treating wood by saturating it with a fireproofing material and an energizer, and then when the same has been by use transformed into charcoal, treating it with a solution of water, sodium carbonate and sodium chlorid thereby to reenergize it. 10  
 19. The process of preparing a carbonizing material which consists in treating sawdust having a fineness adapted to pass through a screen having three or four meshes to the lineal inch by saturating it with a fireproofing material and an energizer, and then when the same has been by use transformed into charcoal, treating it with a solution of water, sodium carbonate and sodium chlorid thereby to reenergize it. 15  
 20. The process of preparing a carbonizing material which consists in treating wood by saturating it with a fireproofing material and an energizer, then when the same has been by use transformed into charcoal, treating it with a solution of water, sodium carbonate and sodium chlorid thereby to energize it, and then retreating it with a similar solution as occasion requires after use thereof to reenergize it. 20  
 21. The process of preparing a carbonizing material which consists in treating sawdust having a fineness adapted to pass through a screen having three or four meshes to the lineal inch by saturating it with a fireproofing material and an energizer, then when the same has been by use transformed into charcoal, treating it with a solution of water, sodium carbonate and sodium chlorid thereby to energize it, and then retreating it with a similar solution as occasion requires after use thereof to reenergize it. 25  
 22. The process of preparing a carbonizing material which consists in treating wood by saturating it with a fire-proofing material and an energizer, then when the same has been by use transformed into charcoal, treating it with a solution of water, sodium carbonate and sodium chlorid in solution of water and about four parts of sodium carbonate to about one of sodium chlorid. 30  
 23. The process of preparing a carbonizing material which consists in treating sawdust of a certain degree of fineness by saturating it with a fireproofing material and an energizer, then when the same has been by use transformed into charcoal, treating it with a solution of water, sodium carbonate and sodium chlorid thereby to energize it, then retreating it with a similar solution as occasion requires after use thereof to reenergize it, then sifting it to remove the deteriorated portions thereof, and then adding a new supply of the previously treated wood or charcoal. 35  
 24. A carbonizing compound consisting of charcoal sprinkled with a liquid solution of salt. 40  
 25. A carbonizing compound consisting of charcoal sprinkled with a liquid solution of soda ash and salt. 45  
 26. A carbonizing compound consisting of a carbonaceous material having applied thereto sodium carbonate, salt and water. 50  
 27. A carbonizing compound consisting in a wood residuum treated with a mixture of soda ash, salt and water in solution. 55  
 28. A carbonizing compound consisting of a fireproofed wood residuum treated with a mixture of soda ash and salt in solution. 60  
 29. A carbonizing compound consisting of a fireproofed and energized wood residuum treated with a mixture of soda ash and salt in solution. 65  
 30. A carbonizing material consisting of a fireproofed and energized wood charcoal treated while hot with water, sodium carbonate and sodium chlorid in solution of water and about four parts of sodium carbonate to about one of sodium chlorid. 70  
 Signed at Cleveland, Ohio, this first day of June, 1917.
- CHARLES PLEASANTS MEBANE.
- Witnesses:
- GEO. R. LAMB,  
W. W. CRAY.

It is hereby certified that in Letters Patent No. 1,310,918, granted July 22, 1919, upon the application of Charles Pleasants Mèbane, of Cleveland, Ohio, for an improvement in "Carbonizing Compounds and Processes of Making the Same," errors appear requiring correction as follows: In the granting clause for "Edwin C. Henn, its successors or assigns" read *Edwin C. Henn, his heirs or assigns*; line 9 of the grant and line 2 of the heading to the printed specification strike out the words "a Corporation of Ohio;" and that the said Letters Patent should be read with these corrections therein that the same may conform to the record of the case in the Patent Office.

Signed and sealed this 19th day of August, A. D., 1919.

[SEAL.]

J. T. NEWTON,  
*Commissioner of Patents.*

Cl. 148—30.